# EUROPEAN PATENT SPECIFICATION

(11) **EP 1 657 335 B1**
(45) Date of publication and mention of the grant of the patent: **06.05.2009**
(21) Application number: 05109326.8
(22) Date of filing: 07.10.2005
(51) Int. Cl.: D04H 3/04, D21F 1/00, D04H 13/00

(54) **Vapour Permeable Clothing**
Wasserdampfdurchlässige Kleidung
Vêtements perméable à la vapeur d'eau

(30) Priority: 12.11.2004 DE 102004054804
(43) Date of publication of application: 17.05.2006
(73) Proprietor: Voith Patent GmbH, 89522 Heidenheim (DE)
(72) Inventor: Morton, Antony, LS298QU, Ben Rhydding (GB)

(56) References cited:
- US-A- 5 585 161

## Description

### FIELD OF INVENTION

The present invention relates to Non-woven fabrics, particular paper machine clothing e.g. as forming fabrics, dryer fabrics or base cloths of press felts.

Paper is conventionally manufactured by conveying a paper furnish, usually consisting of an initial slurry of cellulosic fibres, on a forming fabric or between two forming fabrics in a forming section, the nascent sheet then being passed through a pressing section and ultimately through a drying section of a papermaking machine. In the case of standard tissue paper machines, the paper web is transferred from the press fabric to a Yankee dryer cylinder and then creped.

Paper machine clothing is essentially employed to carry the paper web through these various stages of the papermaking machine. In the forming section the fibrous furnish is wet-laid onto a moving forming wire and water is encouraged to drain from it by means of suction boxes and foils. The paper web is then transferred to a press fabric that conveys it through the pressing section, where it usually passes through a series of pressure nips formed by rotating cylindrical press rolls. Water is squeezed from the paper web and into the press fabric as the web and fabric pass through the nip together. In the final stage, the paper web is transferred either to a Yankee dryer, in the case of tissue paper manufacture, or to a set of dryer cylinders upon which, aided by the clamping action of the dryer fabric, the majority of the remaining water is evaporated.

### DESCRIPTION OF PRIOR ART

Fabrics like Paper machine clothing are mainly manufactured by weaving. The yarns used for weaving can be for example of single or twisted monofilament, multifilament or spun bound type. Materials used are based on polyester, polyamide or polyphenylene sulphide (PPS).

The weaving process is characterized in that the finished fabric comprises interwoven warp and weft yarns, whereby the warp and weft yarns cross over each other at cross-over points resulting in the fact that a woven fabric never can have totally flat surfaces. Therefore fabrics often are characterized by surface features that are predominantly made up of warp or weft dominated arrays.

For some applications it is desirable to have fabrics with flat surfaces. E.g. in the dryer section one function of the dryer fabric is to give sufficient heat transfer from the heated surface e.g. of a drying cylinder to the sheet of paper. This is typically achieved by sandwiching the paper sheet between the dryer fabric and the drying cylinder. The effectiveness of the heat transfer is determined by factors such as pressure applied to press the sheet against the heated cylinder and the contact density (contact area and contact points), that means the contacting surface between the dryer fabric and the sheet.

A drawback of woven fabrics is that they are showing the property of "crimp" caused by the over and under arrangement of the warp and weft yarns. After the weaving process mainly the warp yarns are crimped. During the heat stabilizing process, where heat and tension simultaneously is applied to the fabric, some of the crimp is lost from the warp yarns but imparted into the weft yarns, this is called "crimp interchange".

Fabrics have to exhibit uniform properties for example characterized by their vapour and / or water permeability, caliper, surface topography, tension, dimensional stability etc. through their entire length and width. These properties have to maintain stable over their entire life time. Sometimes the performance of woven fabrics in maintaining properties over their life is not satisfactory.

As a result from the weaving process, the woven fabric has a woven structure with channels for water and vapor passage resulting in a certain water and vapor permeability of the fabric. In the forming and pressing section of a paper making machine mainly the water permeability of the fabric is important to control the liquid dewatering and to avoid rewetting of the sheet. In the dryer section mainly the vapor permeability of the fabric is important to control the passage of moisture vapor from the sheet through the fabric.

Further woven fabrics are not easy to clean because of their complex 3-dimensional open structure. This issue becomes more and more important due to the fact that within the paper making process there is a constant drive towards more and more recycled material to be used including more contaminants. This leads to increased contaminations of the fabric.

To overcome some of the above mentioned drawbacks non woven fabrics have been proposed.

US 3,323,226 describes a synthetic dryer fabric made by mechanical perforating polymeric sheet material.

US 4,541,895 describes a paper makers fabric made up of a plurality of impervious non-woven sheets joined together in a laminated arrangement to define the fabric or belt. Defined throughout the fabric are drainage apertures which are created by drilling techniques.

GB 2 235 705 describes a method for manufacturing a non-woven fabric where an array of sheath core yarns of which the core has a higher melting point than the sheath, is fed in spaced parallel disposition to peripheral grooves of a pinned roller arranged in nip forming relationship with a press roll. Thereby the material of the sheath is melted as the yarns move into and through the roller nip and excess melted sheath material is forced into lateral grooves in the roller to form structural members between adjacent yarns.

From US 5,585,161 a highloft thermally bonded fibre batting with embedded reinforcing yarns is known. According to this document the fibres of the fibre batt are bonded together by low melt fibres.

All the above mentioned non-woven structures are showing unsatisfactory dimensional and thermal stability.

### SUMMARY OF THE INVENTION

It is in general an object of the present invention to provide a non-woven fabric which can be adapted to the requirements of its specific application.

It is an object of the present invention to provide a fabric that has an improved thermal and dimensional stability optionally combined with a high wear resistance.

It is further an object of the present invention to provide an non-woven fabric which can be manufactured more economic than existing non-woven fabrics.

It is in addition an object of the present invention to provide an non-woven fabric whose the permeability can be easy adjusted during manufacturing.

It is another object of the present invention to provide a method of manufacturing an above mentioned non-woven fabric.

According to the present invention there is provided paper machine clothing comprising a non-woven fabric comprising linear yarns spaced apart and extending substantially parallel to each other. The fabric further comprise a matrix structure comprising polymeric matrix material, wherein said matrix structure interconnects and at least partially embeds said yarns. The fabric according to the invention is **characterized in that** said matrix structure comprise filler material incorporated in and mixed with said polymeric matrix material that has in at least one physical and / or chemical property a different behaviour to said polymeric matrix material.

By providing a non-woven fabric comprising a matrix structure comprising a mixture of polymeric matrix material and filler material, wherein the filler material has in at least one physical and / or chemical property a different behaviour to said polymeric matrix material a fabric is created combining advantageous properties of the polymeric matrix material with advantageous properties of the filler material.

Such a fabric can be, depending on the specific choice of the polymeric matrix material and the filler material, adapted to nearly each specific requirement of its application.

With the fabric according to the invention it is further possible to combine materials which for them selves alone are not suitable for use in woven textiles, especially industrial textiles such as paper machine clothing.

By way of example, there are a variety of polymeric materials having excellent wear resistance properties but having no ability to be formed into fibres or yarns. On the other hand there are materials having excellent thermal and dimensional stability but behave poor in wear resistance.

According to the invention it is possible to create a non-woven fabric combining the above mentioned advantageous properties in one single structure, what has not been the case for e.g. woven structures.

To create a non-woven fabric having an enhanced thermal dimensional stability according to a preferred embodiment of the present invention the filler material has a coefficient of linear thermal expansion which is smaller than the coefficient of linear thermal expansion of said polymeric matrix material in the temperature range from 20°C to 160°C.

By providing a non-woven matrix structure which has no crimp with a mixture of polymeric material and filler material having a coefficient of linear thermal expansion which is at typical operation conditions of the fabric smaller than the coefficient of linear thermal expansion of said polymeric matrix a thermal stable fabric with low thermal expansion is provided, because the filler material reduces the thermal expansion of the whole structure.

To improve the wear resistance of the non-woven fabric it is advantageous when the polymeric matrix material has a wear resistance being higher than the wear resistance of said filler material at typical operation conditions. The wear resistance in this case is mainly determined by the polymeric matrix material due to the fact that said filler material is at least mostly incorporated in said polymeric matrix material.

Also the degradation resistance of the non-woven fabric can be improved by choosing a polymeric matrix material having a hydrolytic stability and / or resistance to heat degradation being higher than the hydrolytic stability and / or resistance to heat degradation of said filler material at typical operation conditions.

The filler material can comprise, depending on the specific requirements of the application, particulate filler material and / or fibre filler material.

Depending on the specific application, the length of the fibres of said fibre filler material advantageously can be in the range of 50µm to 500µm, preferably 100µm to 250µm.

Especially to provide a fabric having high thermal dimensional stability it is advantageous when said filler material comprise oligomeric organic material and / or polymeric organic material and / or inorganic particles and / or inorganic fibres.

The oligomeric organic material can comprise Polyhedral Oligomeric Silsesquioxane polymers (POSS).

Further the inorganic particles can comprise alone or in combination nano-clays or inorganic systems based on carbide, e.g. silicon carbide (SiC) or Boron Carbide (B4C/B6C).

The inorganic fibres can comprise alone or in combination: glas, Kevlar or Nomex (polymeric materials available from DuPont). All these materials have a linear coefficient of thermal expansion being lower compared to typical thermoplastic materials. Further these materials showing a high modulus.

A filler material having a high modulus in general serves to enhance at least the cross dimensional stability, e.g. intended cross machine direction, of the matrix structure compared to matrix structures only comprising polymeric matrix material.

Depending on the intended specific application of the non-woven fabric the achieved properties can be influenced by the amount of filler material added to the polymeric matrix material. Experiments performed by the applicant have shown that the properties of the matrix structure can be influenced in a wide range if said matrix structure comprise said filler material in the range of 1 weight% to 80 weight%, preferably 1 weight% to 50 weight%, most preferably 5 weight% to 30 weight%.

To generate a homogenous matrix structure having the same chemical and / or physical properties along its entire extension according to a preferred embodiment of the present invention it is foreseen that the filler material is homogenous mixed with said polymeric matrix material.

To achieve a matrix structure with spatial changing physical and / or chemical properties it is desirable, if the matrix structure comprise at least one area having a content of filler material being different to another area and / or comprising filler material being different to the filler material of said another area.

The best results in respect to thermal dimensional stability for the use in the papermaking industry will be achieved if said matrix structure has a coefficient of linear thermal expansion ranging from 1 x 10⁻⁵K⁻¹ to 5 x 10⁻⁵K⁻¹ for temperature range encountered on a paper machine (20°C up to 160°C). This leads to a fabric having a thermal expansion of less than 0,5% when heated from 20°C to 120°C, compared to a non-woven fabric known in the art and made of typical thermoplastic elastomer material which expands in the range of 2% when heated the same amount.

According to a further embodiment of the present invention the polymeric matrix material has a melting temperature being lower than the melting temperature of said linear yarns and / or than the melting temperature of said filler material.

For use in a variety of applications it is necessary that the fabric maintains its dimensions when subjected to pressure. In many applications e.g. in the press section of a papermaking machine the non-woven fabric will be subjected to pressure. To maintain its dimension when subjected to pressure according to a preferred embodiment of the present invention the matrix structure is almost non-deformable. The expression non-deformable can be explained by way of example. In the case of a non-woven fabric having apertures for being permeable to water squeezed out of the paper web in the press section of a paper making machine non-deformable has to be understood that any deformation that may take place during application of pressure would be minimal such that fluid passageways contained within the non-deformable matrix structure would remain open, thereby continuing to provide void space for the accommodation of fluid even under high pressure loading conditions.

For cost efficient processing of the non-woven fabric, e.g using extrusion processes or injection molding processes, the polymeric matrix material has to have thermoplastic properties. Therefore according to a further preferred embodiment of the invention the polymeric matrix material comprise alone or in combination: thermoplastic or thermoplastic elastomer material.

The thermoplastic elastomer material for example can be any type of thermoplastic elastomer based on polyester, polyurethane, polyamide, rubber (organic or inorganic).

Thermoplastics such as polyurethanes or polyesters or polyamides or rubbers can be used for the polymeric matrix material depending on the requirements of the specific application of the fabric. Rubbers could be based on organic systems (such as EPDM types) or inorganic systems (such as Silicone types).

To increase length dimensional e.g. intended machine direction stability of the fabric according to a preferred embodiment of the present invention the linear yarns embedded in the matrix structure have a high modulus. Materials showing a high modulus and a low coefficient of linear thermal expansion are for example glas or Kevlar or Nomex.

According to a further embodiment of the invention the linear yarns are monofilament or multifilament or plied or twisted or spun bond yarns.

Depending on the specific requirements of the intended application of the non-woven fabric it is advantageous if the matrix structure forms a flat surface on at least one face of said non-woven fabric. A fabric having a flat surface on at least one surface is for example needed in the forming and dryer section. In the first case to reduce wire making on the sheet. In the second case in addition for example to provide a maximum contact area between the paper sheet and the drying cylinder to achieve maximum heat transfer between the drying cylinder and the sheet. Further unwanted air carriage of the moving fabric is reduced on the flat surface. This is an important feature due to the fact of continuously increasing paper machine speeds.

For other purposes, for example in the tissue paper making process it is desirable to create a patterned structure onto the tissue sheet. For this application according to a preferred embodiment of the invention the matrix structure forms a textured surface on at least one face of said non-woven fabric.

For some applications e.g. smoothing or transfer belts where no water has to be removed from the paper sheet there is no need for the fabric of being permeable. For other applications where water and / or vapour has to be removed from the sheet the non-woven fabric must have a certain permeability. Therefore the non-woven fabric comprise apertures extending through said matrix structure.

To achieve a certain required permeability the apertures can have any thinkable geometrical shape like straight through holes or conical holes. Further the apertures can extend substantially perpendicular to the general plain of the fabric. The shape of the apertures is also an important factor in regard to the ability of being cleaned. Therefore when designing the apertures the cleaning ability also can be taken into consideration.

For designing the apertures all the above mentioned factors can be considered without the limited flexibility being inherent to woven structures.

To achieve a uniform drainage characteristic throughout the non-woven fabric it is advantageous if the apertures are uniformly spaced.

To achieve a non-uniform, that means zonal different, drainage characteristic throughout the non-woven fabric it is advantageous if the apertures are not uniformly spaced.

For some application esp. to avoid hydraulic marking it is advantageous if the apertures are randomly spaced by maintaining a uniform permeability all over the non-woven fabric.

According to a further embodiment of the invention depending on the specific application the apertures can be straight through holes or conical holes or posses a tortuous, non linear path through the z direction of the structure. Therefore any geometric design suitable for the specific application is possible.

Further the apertures are in laterally offset disposition relative to said linear yarns.

Depending on the distribution, the size and the shape of the apertures a wide range of permeability can be adjusted. The fabric according to the invention therefore can have a permeability in the range of 20cfm to 1000cfm, which can be selected according to the specific requirements of its intended application.

To mostly prevent the load bearing linear extending yarns from the environmental conditions the fabric being subjected during its operation it is advantageous if the linear yarns are fully embedded in said matrix structure.

A plurality of said non-woven fabrics can be joined together in a face to face manner to generate a laminated structure comprising a plurality of such non-woven fabrics. To generate a structure having a width being greater as the width of one of said non-woven fabrics said non-woven fabrics can be joined together in a side by side manner.

If the paper machine clothing is for example a press felt it is possible that at least one surface of said non-woven fabric is covered by a porous layer. This porous layer can for example form the sheet contacting surface of the paper machine clothing.

Further the porous layer can comprise a textile batt and / or foam material.

One of the big advantages of the present invention is that, due to the fact that the non-woven fabric comprise linear spaced apart extending yarns at least partially embedded in a matrix structure, wherein said matrix structure comprise a mixture of a polymeric matrix material and a filler material, wherein said filler material has in at least one physical and / or chemical property a different behaviour to said polymeric matrix material, that said non-woven fabric is applicable for almost all applications in a paper machine. Therefore according to a preferred embodiment of the present invention the paper machine clothing comprising said non-woven fabric can be a forming or dryer fabric, a press felt or press belt, a smoothing or transfer belt.

The invention also includes a method of manufacturing a paper machine clothing, the clothing comprising a non-woven fabric, the manufacturing of the non-woven fabric comprising the steps of forming a matrix structure comprising filler material and polymeric matrix material and applying spaced appart linear yarns substantially extending parallel to each other during or after formation of said matrix structure at a molten stage of said polymeric matrix material in such a way to said matrix structure that said yarns are at least in part embedded into said matrix structure and interconnected by said matrix structure.

To manufacture a non-woven fabric according to the invention having apertures extending through the matrix structure said apertures can be provided by drilling. Apertures can be provided by mechanical drilling/punching methods. Also blasting methods such as water jet or particulate (grit). Apertures also created by ablative process, such as that produced by laser. The laser for ablation can be a CO2 or Nd:YAG laser.

It is further possible to provide the apertures during the manufacturing step producing the matrix structure. Therefore the method can further comprise the steps of applying said spaced apart yarns to a mixture comprising molten polymeric material and filler material, constraining subsequent flow movement of said mixture of polymeric and filler material to predetermined paths extending between and cross linking adjacent yarns to form said non-woven fabric with apertures.

Alternatively core/sheath yarns can be used to produce the non-woven fabric according to the invention. The core/sheath yarns can be made by extrusion techniques producing a core/sheath yarn having a monofilament core and a sheath comprising polymeric material mixed with filler material. In this case the method further comprises the steps of providing spaced apart sheath/core yarns, each of said sheath/core yarns comprising a core yarn and a sheath, the sheath comprising polymeric material mixed with filler material, heating the sheath/core yarns to melt said polymeric material, constraining subsequent flow movement of said mixture of polymeric and filler material to predetermined paths extending between and cross linking said adjacent core yarns to form said non-woven fabric with apertures.

By doing this a non-woven fabric having apertures is formed, wherein the core yarns form the linear extending spaced apart reinforcing yarns being embedded in a matrix structure comprising polymeric matrix material and filler material, being provided by the sheath material.

Further the method can comprise that the flow movement of the mixture of polymeric and filler material is constrained to individual paths arranged in spaced apart disposition in the longitudinal direction of said yarns.

The predetermined paths can be provided by a pinned drum.

To guaranty the full formation and proper distribution of the polymeric material mixed with the filler material according to a preferred embodiment of the present invention it is foreseen that the flow movement of the mixture of polymeric and filler material is influenced by pressure applied to the mixture of polymeric and filler material perpendicular to the flow moving directions.

The pressure can be provided by a press-nip formed between the pinned drum and a press roll or a doctor blade.

In order that the present invention may be more readily understood, specific embodiments will now be described with reference to the accompanying drawings in which:
- Fig. 1: is a top view onto a part of a non-woven fabric according to a first embodiment of the invention;
- Fig. 2: is a side view of the non-woven fabric of fig. 1;
- Fig. 3: is a top view onto a part of a non-woven fabric according to a second embodiment of the invention; and
- Fig. 4: is a side view of an apparatus to perform the method according to the invention.
- Fig. 5: is a cross sectional view on a core/sheath yarn.

Fig. 1 is showing a view onto a face 7 of a part of a non-woven fabric 1 of a paper machine clothing according to a first embodiment of the invention. The non-woven fabric 1 shown in Fig. 1 is for the use in a paper machine.

The non-woven fabric 1 comprise apertures 6 extending through the fabric 1 and being uniformly spaced. In the specific embodiment of Fig. 1 the apertures 6 are conical holes giving the fabric 1 a permeability of 750cfm. For sure the scope of the invention is not limited to conical holes. Depending on the specific application any thinkable geometry could be used. also the permeability depends on the specific application requirement and can be in the range of 20cfm to 1000cfm.

The apertures 6 provide individual flow passages substantially perpendicular to the general plane of the fabric 1 lying in the plane of the drawing.

The non-woven fabric 1 comprise linear spaced apart yarns 2 extending substantially parallel to each other. The yarns are monofilament yarns 2 made from extruded and drawn thermoplastic material. This is most typically based on polyester for dryer application. For other parts of the paper machine one could envisage polyamide based. Exotic materials such as PPS (polyphenylene sulphide) and PEEK (polyetherether ketone) could also be used. For applications other than for the dryer section it may be possible to use multifilament, spun, glass reinforced plied yarns etc..

Further the non-woven fabric comprise a matrix structure 3 comprising polymeric matrix material 4 and filler material 5 mixed with said polymeric matrix material 4. The matrix structure 3 forms a flat surface on face 7 of said non-woven fabric 1.

The apertures 6 are provided in the matrix structure 3. Further the apertures 6 are in laterally offset disposition relative to the linear yarns 2.

The matrix structure 3 interconnects and fully embeds the yarns 2. The yarns 2 extend in the intended machine direction (MD) of the fabric 1 and serve as reinforcing yarns.

The filler material 5 of the specific embodiment shown in Fig. 1 is in fibre 5 form and has according to the invention in at least one physical and / or chemical property a different behaviour to the polymeric matrix material 4.

In the embodiment shown in Fig. 1 the fibres 5 providing the filler material 5 has a coefficient of linear thermal expansion which is smaller than the coefficient of thermal expansion of said polymeric matrix material in the temperature range typical in paper machines. The fibres 5 are glas fibres. The fibres 5 in the specific embodiment shown in Fig. 1 have a length distribution in the range from 100µm to 250µm. It also could have been possible to select fibres only having one specific length. Further the fibres 5 are added to the polymeric material 4 so that the matrix structure 3 comprise the fibres 5 in an amount in the range of 25 weight%.

Further the fibres 5 are homogenous distributed in the polymeric matrix material 4. Further the fibres 5 have non preferred orientation in the polymeric matrix material 4 so that the matrix structure 3 has an isotropic behaviour in its properties. It also could have been possible to provide the fibres 5 with a preferred orientation to give the matrix structure 3 an anisotropic behaviour.

Further the polymeric matrix material 4 has a wear resistance being higher than the wear resistance of the filler material 5. In the specific embodiment shown in Fig. 1 the polymeric matrix material 4 comprise polyurethane which has an excellent wear resistance. For application in the dryer section the it is advantageous if the polymeric matrix material 4 comprise or is a thermoplastic elastomer based material.

The matrix structure 3 comprising said polymeric material 4 mixed with said fibres has a coefficient of linear thermal expansion ranging from 1 x 10⁻⁵K⁻¹ to 5 x 10⁻⁵K⁻¹ over the temperature range typically encountered within a paper making machine. This leads to an expansion of the non-woven fabric 1 when heated from 20°C to 120°C of around 0,5%.

By way of comparison polyurethane for its alone (without filler) has a coefficient of linear thermal expansion of greater than 1 x 10⁻⁴ K⁻¹, leading to an expansion of the non-woven fabric when exposed to the full temperature range likely to be encountered on a paper making machine of around 2,0%.

Therefore the fabric 1 according to the invention has a increased thermal dimensional stability.

Further the polymeric matrix material 4 has a melting temperature being lower than the melting temperature of the linear yarns 2 and the melting temperature of the filler fibres 5. In addition the fibres 5 and the yarns 2 have a higher modulus than the polymeric matrix material 4. Typical values for the modulus are for example 50-100GPa for glass and 0,02-4GPa for thermoplastics and thermoplastic elastomers.

Referring now to Fig. 2 which shows a cross sectional view of the non-woven fabric 1 along the line A-A cutting through the apertures 6.

As can be seen the matrix structure 3 forms flat surfaces on faces 7 and 8 of the non-woven fabric 1.

In Fig. 2 the yarns 2 extend perpendicular to the plane of drawing.

Apertures 6 extend through the matrix structure 3 and showing a conical / tapered shape.

Fig. 3 is showing a view onto a face 15 of a part of a non-woven fabric 10 according to a second embodiment of the invention. The non-woven fabric 10 shown in Fig. 3 is for the use in a paper machine clothing e.g. as a transfer belt.

The non-woven fabric 10 comprise no apertures and therefore is not permeable. Further the non-woven fabric 10 comprise linear spaced apart yarns 11 extending substantially parallel to each other. The yarns 11 are monofilament yarns and made from thermoplastic polyester (PET) that has been extruded and drawn.

Further the non-woven fabric comprise a matrix structure 12 comprising polymeric matrix material 13 and filler material 14 mixed with said polymeric matrix material 13. The matrix structure 12 forms a flat surface on face 15 of said non-woven fabric 10.

The matrix structure 12 interconnects and fully embeds the yarns 11. The yarns 11 extend in the intended machine direction (MD) of the fabric 10 and serve as reinforcing yarns.

The filler material 14 of the specific embodiment shown in Fig. 3 is in particulate form and has according to the invention in at least one physical and / or chemical property a different behaviour to the polymeric matrix material 13.

In the embodiment shown in Fig. 3 the particles 14 providing the filler material 14 have an abrasion resistance which is lower than that of said polymeric matrix material 13. The particles 14 comprise SiC. It also could have been that all the particles would have one specific particle size selected from the above mentioned range. Further the particles 14 are added to the polymeric material 13 so that the matrix structure 12 comprise the particles 14 in an amount in the range of 20 weight%.

Further the particles 14 are homogenous distributed in the polymeric matrix material 13.

In the specific embodiment shown in Fig. 3 the polymeric matrix material 13 comprise thermoplastic elastomer based on polyester.

It has to be understood that the invention also embodiments having particulate filler material in a matrix structure having apertures. Also it has to be understood that the invention covers embodiments having fibre filler material in a matrix structure having no apertures.

Fig. 4 shows a cross sectional side view of an apparatus 20 to perform the method of manufacturing a non-woven fabric 21 according to the invention.

An array of linear spaced apart core/sheath yarns 22 is fed onto a rotating pinned drum 27. Each of said yarns 22 have a sheath 23 comprising a mixture of polymeric material 24 and filler material 25 embedding a polymeric core yarn 26. The polymeric material 24 has a melting temperature which is lower than the melting temperature of the filler material 25 and of the core yarns 26. The core/sheath yarns 22 are heated by a heating supply 28 to melt the polymeric material 24 without melting the filler material 25 and the core yarn 26.

The core/sheath yarns 22 can be melted by direct impingement of electromagnetic radiation (infra-red, microwave etc ...) or they can be melted through an induction effect whereby the surface temperature of the pin-drum 27 is raised by an induction heater to a temperature that is above the melting temperature of the sheath material 24, but below the melting temperature of the core yarns 26 or the filler material 25.

The molten polymeric material 24 and the filler material 25 is subjected to pressure provided by a press-nip 29 formed by the pinned drum 27 and a press roll 30.

The pressure is applied perpendicular to the intended flow movement direction of the mixture of the molten polymeric material 24 and filler material 25 and forces mixture 24 and 25 to flow along predetermined paths 31, provided by the pinned drum 27, to extend between and to cross link adjacent core yarns 26. Further the pressure forces the mixture of molten polymeric material 24 and filler material 25 to flow along individual paths in the longitudinal direction of the core yarns 26. The paths are provided by the pinned drum 27 and arranged in spaced apart disposition.

By doing this, the non-woven fabric 21 is formed, wherein said core yarns 26 provides aforesaid yarns 2 and / or 11, said polymeric material 24 provides aforesaid polymeric matrix material 4 and / or 13 and said filler material provides aforesaid filler material 5 and / or 14 described in Fig.'s 1, 2 and 3.

Fig. 5 is showing a cross sectional view of the core/sheath yarn 22 used to perform the method described above. The core/sheath yarn has been manufactured by a conventional extrusion technique.

As can be seen the core/sheath yarn has a core 26 being fully embedded in a sheath 23. The sheath 23 comprises a mixture of polymeric material 24 and filler material 25. The polymeric material 24 has a melting temperature which is lower than the melting temperature of the filler material 25 and of the core yarns 26.

While the invention has been described in detail, it will be apparent to one skilled in the art that various changes and modifications can be made therein without departing from the scope thereof.

## Claims

1. Paper machine clothing comprising at least one non-woven fabric (1, 10), the non-woven fabric (1, 10) comprising linear yarns (2, 11) spaced apart and extending substantially parallel to each other and a matrix structure (3, 12) comprising polymeric matrix (4, 13) material, wherein said matrix structure (3, 12) interconnects and at least partially embeds said yarns (2, 11), wherein said matrix structure (3, 12) comprise filler material (5, 14) incorporated in and mixed with said polymeric matrix material (4, 13), wherein said filler material (5, 14) has in at least one physical and / or chemical property a different behaviour to said polymeric matrix material (4, 13).

2. Paper machine clothing according to claim 1,
**characterized in**
**that** said filler material (5, 14) has a coefficient of linear thermal expansion which is smaller than the coefficient of thermal expansion of said polymeric matrix material (4, 13) at least in a temperature range from 20°C to 160°C.

3. Paper machine clothing according to claim 1 or 2,
**characterized in**
**that** said polymeric matrix material (4, 13) has a wear resistance being higher than the wear resistance of said filler material (5, 14).

4. Paper machine clothing according to one of the claims 1 to 3,
**characterized in**
**that** said polymeric matrix material (4, 13) having a hydrolytic stability and / or resistance to heat degradation being higher than the hydrolytic stability and / or resistance to heat degradation of said filler material (5, 14).

5. Paper machine clothing according to one of the claims 1 to 4,
**characterized in**
**that** said filler material (5, 14) comprise particulate filler material (14) and / or fibre filler material (5).

6. Paper machine clothing according to claim 5,
**characterized in**
**that** the fibres of said fibre filler material (5) have a length in the range of 50µm to 500µm, preferably 100µm to 250µm.

7. Paper machine clothing according to one of the preceding claims,
**characterized in**
**that** said filler material (5, 14) comprise oligomeric organic material and / or polymeric organic material and / or inorganic particles and / or inorganic fibres.

8. Paper machine clothing according to claim 7,
**characterized in**
**that** said oligomeric organic material comprise Polyhedral Oligomeric Silsesquioxane polymers.

9. Paper machine clothing according to claim 7,
**characterized in**
**that** said inorganic particles comprise nano-clays and / or SiC and / or Boron Carbide.

10. Paper machine clothing according to one of the claims 7 to 9,
**characterized in**
**that** said inorganic fibres comprise alone or in combination: glas, Kevlar or Nomex.

11. Paper machine clothing according to one of the preceding claims,
**characterized in**
**that** said matrix structure comprise said filler material (5, 14) in the range of 1 weight% to 80 weight%, preferably 1 weight% to 50 weight%, most preferably 5 weight% to 30 weight%.

12. Paper machine clothing according to one of the preceding claims,
**characterized in**
**that** said matrix structure comprise said fibre filler material (5) in the range of 5-20 weight %, preferably 8-12 weight %.

13. Paper machine clothing according to one of the preceding claims,
**characterized in**
**that** said matrix structure comprise said particulate filler material (14) in the range of 5-50 weight %, preferably 10-30 weight %.

14. Paper machine clothing according to one of the preceding claims,
**characterized in**
**that** said filler material (5, 14) is homogenous mixed in said polymeric matrix material (4, 13).

15. Paper machine clothing according to one of the claims 1 to 14,
**characterized in**
**that** said matrix structure comprise at least one area with a content of filler material (5, 14) being higher compared to an other area.

16. Paper machine clothing according to one of the preceding claims,
**characterized in**
**that** said matrix structure comprising filler material (5, 14) has a coefficient of linear thermal expansion ranging from 1 x 10⁻⁵K⁻¹ to 5 x 10⁻⁵K⁻¹.

17. Paper machine clothing according to one of the preceding claims,
**characterized in**
**that** said polymeric matrix material (4, 13) has a melting temperature being lower than the melting temperature of said linear yarns and / or than the melting temperature of said filler material (5, 14).

18. Paper machine clothing according to one of the preceding claims,
**characterized in**
**that** said polymeric matrix material (4, 13) comprise alone or in combination: thermoplastic or thermoplastic elastomer material such as thermoplastic elastomer based polyester, polyurethane, polyamide, rubber (organic or inorganic).

19. Paper machine clothing according to one of the preceding claims,
**characterized in**
**that** said linear yarns (2, 11) are monofilament or multifilament or plied or twisted or spun bond yarns.

20. Paper machine clothing according to one of the preceding claims ,
**characterized in**
**that** said linear yarns (2, 11) comprise inorganic material.

21. Paper machine clothing according to one of the preceding claims,
**characterized in**
**that** said matrix structure (3, 12) forms a flat surface on at least one face of said non-woven fabric.

22. Paper machine clothing according to one of the preceding claims,
**characterized in**
**that** said matrix structure (3, 12) forms a textured surface on at least one face of said Paper machine clothing.

23. Paper machine clothing according to one of the preceding claims,
**characterized in**
**that** said non-woven fabric comprise apertures (6) extending through said matrix structure(3, 12).

24. Paper machine clothing according to claim 25,
**characterized in**
**that** said apertures (6) are uniformly spaced.

25. Paper machine clothing according to one of the claims 25 to 26,
**characterized in**
**that** said apertures (6) are in laterally offset disposition relative to said linear yarns.

26. Paper machine clothing according to one of claims 25 to 27,
**characterized in**
**that** said apertures (6) are straight through holes or conical holes.

27. Paper machine clothing according to one of the preceding claims,
**characterized in**
**that** said fabric has a permeability in the range of 20cfm to 1000cfm (9,43894x10⁻³m³/s to 0,471947m³/s).

28. Paper machine clothing according to one of the preceding claims,
**characterized in**
**that** said apertures (6) in the matrix structure (3, 12) comprise respective individual flow passages substantially perpendicular to the general plane of said fabric.

29. Paper machine clothing according to one of the preceding claims,
**characterized in**
**that** said linear yarns (2, 11) are fully embedded in said matrix structure(3, 12).

30. Paper machine clothing according to to one of the preceding claims,
**characterized in**
**that** said paper machine clothing comprise a plurality of said non-woven fabrics (1, 10) joined together in a laminated and / or side by side manner.

31. Paper machine clothing according to to one of the preceding claims,
**characterized in**
**that** at least one surface of said non-woven fabric is covered by a porous layer.

32. Paper machine clothing according to to one of the preceding claims,
**characterized in**
**that** said porous layer comprise a textile batt.

33. Paper machine clothing according to to one of the preceding claims,
**characterized in**
**that** said paper machine clothing is a forming or dryer fabric, a press felt or press belt, a smoothing or transfer belt.

34. Method of manufacturing a paper machine clothing with a non-woven fabric, the method comprising the steps of forming a matrix structure comprising filler material and polymeric matrix material and applying spaced appart linear yarns substantially extending parallel to each other during or after formation of said matrix structure at a molten stage of said polymeric matrix material in such a way to said matrix structure that said yarns are at least in part embedded into said matrix structure and interconnected by said matrix structure.

## Patentansprüche

1. Papiermaschinenbespannung, umfassend ein nicht durch Weben entstandenes textiles Flächengebilde (1, 10) mit voneinander beabstandeten und im wesentlichen parallel zueinander verlaufenden linearen Fäden (2, 11) und einer wenigstens teilweise aus einer Polymermatrixmasse (4, 13) bestehenden Matrixstruktur (3, 12), wobei die Fäden (2, 11) durch die Matrixstruktur (3, 12) miteinander verbunden und mindestens teilweise darin eingebettet sind, wobei die Matrixstruktur (3, 12) wenigstens teilweise aus einer mit der Polymermatrixmasse (4, 13) vermischten Füllmasse (5, 14) besteht, wobei die Füllmasse (5, 14) sich in mindestens einer physikalischen und/oder chemischen Eigenschaft von der Polymermatrixmasse (4, 13) unterscheidet.

2. Papiermaschinenbespannung nach Anspruch 1, **dadurch gekennzeichnet, daß** die Füllmasse (5, 14) zumindest in einem Temperaturbereich von 20°C bis 160°C einen kleineren linearen Wärmeausdehnungskoeffizienten als die Polymermatrixmasse (4, 13) aufweist.

3. Papiermaschinenbespannung nach Anspruch 1 oder 2, **dadurch gekennzeichnet, daß** die Polymermatrixmasse (4, 13) eine höhere Verschleißfestigkeit als die Füllmasse (5, 14) aufweist.

4. Papiermaschinenbespannung nach einem der Ansprüche 1 bis 3, **dadurch gekennzeichnet, daß** die Polymermatrixmasse (4, 13) eine höhere Hydrolysebeständigkeit und/oder Wärmeabbauresistenz als die Füllmasse (5, 14) aufweist.

5. Papiermaschinenbespannung nach einem der Ansprüche 1 bis 4, **dadurch gekennzeichnet, daß** die Füllmasse (5, 14) wenigstens teilweise aus teilchenförmiger Füllmasse (14) und/oder faserförmiger Füllmasse (5) besteht.

6. Papiermaschinenbespannung nach Anspruch 5, **dadurch gekennzeichnet, daß** die faserförmige Füllmasse (5) eine Faserlänge von 50 µm bis 500 µm und bevorzugt 100 µm bis 250 µm aufweist.

7. Papiermaschinenbespannung nach einem der vorhergehenden Ansprüche, **dadurch gekennzeichnet, daß** die Füllmasse (5, 14) wenigstens teilweise aus oligomerem organischem Material und/oder polymerem organischem Material und/oder anorganischen Teilchen und/oder anorganischen Fasern besteht.

8. Papiermaschinenbespannung nach Anspruch 7, **dadurch gekennzeichnet, daß** das oligomere organische Material wenigstens teilweise aus polyedrischen oligomeren Silasesquioxanpolymeren besteht.

9. Papiermaschinenbespannung nach Anspruch 7, **dadurch gekennzeichnet, daß** die anorganischen Teilchen wenigstens teilweise aus Nanotonen und/oder SiC und/oder Borcarbid bestehen.

10. Papiermaschinenbespannung nach einem der Ansprüche 7 bis 9, **dadurch gekennzeichnet, daß** die anorganischen Fasern wenigstens teilweise aus Glas, Kevlar oder Nomex allein oder in Kombination bestehen.

11. Papiermaschinenbespannung nach einem der vorhergehenden Ansprüche, **dadurch gekennzeichnet, daß** die Matrixstruktur die Füllmasse (5, 14) in einem Anteil von 1 Gew.-% bis 80 Gew.-%, bevorzugt 1 Gew.-% bis 50 Gew.-% und ganz besonders bevorzugt 5 Gew.-% bis 30 Gew.-% enthält.

12. Papiermaschinenbespannung nach einem der vorhergehenden Ansprüche, **dadurch gekennzeichnet, daß** die Matrixstruktur die faserförmige Füllmasse (5) mit 5-20 Gew.-% und bevorzugt 8-12 Gew.-% enthält.

13. Papiermaschinenbespannung nach einem der vorhergehenden Ansprüche, **dadurch gekennzeichnet, daß** die Matrixstruktur die teilchenförmige Füllmasse (14) mit 5-50 Gew.-% und bevorzugt 10-30 Gew.-% enthält.

14. Papiermaschinenbespannung nach einem der vorhergehenden Ansprüche, **dadurch gekennzeichnet, daß** die Polymermatrixmasse (4, 13) die Füllmasse (5, 14) homogen eingemischt enthält.

15. Papiermaschinenbespannung nach einem der Ansprüche 1 bis 14, **dadurch gekennzeichnet, daß** die Matrixstruktur mindestens einen Bereich mit einem höheren Gehalt an Füllmasse (5, 14) als in einem anderen Bereich aufweist.

16. Papiermaschinenbespannung nach einem der vorhergehenden Ansprüche, **dadurch gekennzeichnet, daß** die Matrixstruktur wenigstens teilweise aus Füllmasse (5, 14) mit einem linearen Wärmeausdehnungskoeffizienten von 1x10⁻⁵ K⁻¹ bis 5x10⁻⁵ K⁻¹ besteht.

17. Papiermaschinenbespannung nach einem der vorhergehenden Ansprüche, **dadurch gekennzeichnet, daß** die Polymermatrixmasse (4, 13) einen Schmelzpunkt aufweist, der unter dem Schmelzpunkt der linearen Fäden und/oder dem Schmelzpunkt der Füllmasse (5, 14) liegt.

18. Papiermaschinenbespannung nach einem der vorhergehenden Ansprüche, **dadurch gekennzeichnet, daß** die Polymermatrixmasse (4, 13) wenigstens teilweise aus thermoplastischem oder thermoplastisch-elastomerem Material wie auf thermoplastischem Elastomer basierendem Polyester, Polyurethan, Polyamid, Gummi (organisch oder anorganisch) allein oder in Kombination besteht.

19. Papiermaschinenbespannung nach einem der vorhergehenden Ansprüche, **dadurch gekennzeichnet, daß** es sich bei den linearen Fäden (2, 11) um monofile oder multifile oder gefachte oder gedrehte oder Spinngarne handelt.

20. Papiermaschinenbespannung nach einem der vorhergehenden Ansprüche, **dadurch gekennzeichnet, daß** die linearen Fäden (2, 11) wenigstens teilweise aus anorganischem Material bestehen.

21. Papiermaschinenbespannung nach einem der vorhergehenden Ansprüche, **dadurch gekennzeichnet, daß** die Matrixstruktur (3, 12) auf mindestens einer Seite des nicht durch Weben entstandenen textilen Flächengebildes eine flache Oberfläche bildet.

22. Papiermaschinenbespannung nach einem der vorhergehenden Ansprüche, **dadurch gekennzeichnet, daß** die Matrixstruktur (3, 12) auf mindestens einer Seite der Papiermaschinenbespannung eine strukturierte Oberfläche bildet.

23. Papiermaschinenbespannung nach einem der vorhergehenden Ansprüche, **dadurch gekennzeichnet, daß** das nicht durch Weben entstandene textile Flächengebilde durch die Matrixstruktur (3, 12) hindurchreichende Öffnungen (6) umfaßt.

24. Papiermaschinenbespannung nach Anspruch 25, **dadurch gekennzeichnet, daß** die Öffnungen (6) einheitlich voneinander beabstandet sind.

25. Papiermaschinenbespannung nach einem der Ansprüche 25 bis 26, **dadurch gekennzeichnet, daß** die Öffnungen (6) gegenüber den linearen Fäden seitlich versetzt angeordnet sind.

26. Papiermaschinenbespannung nach einem der Ansprüche 25 bis 27, **dadurch gekennzeichnet, daß** es sich bei den Öffnungen (6) um gerade Durchgangslöcher oder konische Löcher handelt.

27. Papiermaschinenbespannung nach einem der vorhergehenden Ansprüche, **dadurch gekennzeichnet, daß** es eine Durchlässigkeit von 20 cfm bis 1000 cfm (9,43894×10⁻³m³/s bis 0,471947m³/s) aufweist.

28. Papiermaschinenbespannung nach einem der vorhergehenden Ansprüche, **dadurch gekennzeichnet, daß** die Öffnungen (6) in der Matrixstruktur (3, 12) jeweils einzelne im wesentlichen senkrecht zur allgemeinen Ebene des textilen Flächengebildes verlaufende Strömungskanäle umfassen.

29. Papiermaschinenbespannung nach einem der vorhergehenden Ansprüche, **dadurch gekennzeichnet, daß** die linearen Fäden (2, 11) vollständig in der Matrixstruktur (3, 12) eingebettet sind.

30. Papiermaschinenbespannung nach einem der vorhergehenden Ansprüche, **dadurch gekennzeichnet, daß** sie wenigstens teilweise aus mehreren der nicht durch Weben entstandenen textilen Flächengebilde (1, 10) besteht, die in einem Laminat und/oder Seite an Seite miteinander verbunden sind.

31. Papiermaschinenbespannung nach einem der vorhergehenden Ansprüche, **dadurch gekennzeichnet, daß** das nicht durch Weben entstandene textile Flächengebilde mindestens einseitig mit einer porösen Schicht bedeckt ist.

32. Papiermaschinenbespannung nach einem der vorhergehenden Ansprüche, **dadurch gekennzeichnet, daß** die poröse Schicht mindestens teilweise aus einer textilen Vlieslage besteht.

33. Papiermaschinenbespannung nach einem der vorhergehenden Ansprüche, **dadurch gekennzeichnet, daß** es sich dabei um ein Formier- oder Trockensieb, einen Preßfilz oder ein Preßband oder ein Glätt- oder Transferband handelt.

34. Verfahren zur Herstellung einer Papiermaschinenbespannung mit einem nicht durch Weben herzustellenden textilen Flächengebilde, bei dem man eine wenigstens teilweise aus Füllmasse und Polymermatrixmasse bestehende Matrixstruktur bildet und darauf im geschmolzenen Zustand der Polymermatrixmasse während oder nach Bildung der Matrixstruktur lineare Fäden voneinander beabstandet und im wesentlichen parallel zueinander verlaufend so aufbringt, daß die Fäden mindestens zum Teil darin eingebettet und **dadurch** miteinander verbunden sind.

## Revendications

1. Habillage de machine à papier comprenant au moins une toile non tissée (1, 10), la toile non tissée (1, 10) comprenant des fils linéaires (2, 11) espacés et s'étendant essentiellement de manière parallèle les uns des autres, et une structure matricielle (3, 12) comprenant un matériau de matrice polymère (4, 13), dans lequel ladite structure matricielle (3, 12) s'interconnecte et s'intègre au moins partiellement auxdits fils (2, 11), dans lequel ladite structure matricielle (3, 12) comprend un matériau de charge (5, 14) incorporé dans et mélangé audit matériau de matrice polymère (4, 13), dans lequel ledit matériau de charge (5, 14) possède un comportement différent dudit matériau de matrice polymère (4, 13) dans au moins une propriété physique et/ou chimique.

2. Habillage de machine à papier selon la revendication 1, **caractérisé en ce que** ledit matériau de charge (5, 14) possède un coefficient de dilatation thermique linéaire qui est inférieur au coefficient de dilatation thermique dudit matériau de matrice polymère (4, 13) au moins dans la plage de températures de 20 °C à 160 °C.

3. Habillage de machine à papier selon la revendication 1 ou la revendication 2, **caractérisé en ce que** ledit matériau de matrice polymère (4, 13) possède une résistance à l'usure supérieure à la résistance à l'usure dudit matériau de charge (5, 14).

4. Habillage de machine à papier selon l'une des revendications 1 à 3, **caractérisé en ce que** ledit matériau de matrice polymère (4, 13) possède une stabilité hydrolytique et/ou une résistance à la dégradation thermique supérieure à la stabilité hydrolytique et/ou à la résistance à la dégradation thermique dudit matériau de charge (5, 14).

5. Habillage de machine à papier selon l'une des revendications 1 à 4, **caractérisé en ce que** ledit matériau de charge (5, 14) comprend un matériau de charge particulaire (14) et/ou un matériau de charge fibreux (5).

6. Habillage de machine à papier selon la revendication 5, **caractérisé en ce que** les fibres dudit matériau de charge fibreux (5) ont une longueur dans la plage de 50 µm à 500 µm, de préférence de 100 µm à 250 µm.

7. Habillage de machine à papier selon l'une des revendications précédentes, **caractérisé en ce que** ledit matériau de charge (5, 14) comprend un matériau organique oligomère et/ou un matériau organique polymère et/ou des particules inorganiques et/ou des fibres inorganiques.

8. Habillage de machine à papier selon la revendication 7, **caractérisé en ce que** ledit matériau organique oligomère comprend des polymères de silsesquioxane oligomère polyédrique.

9. Habillage de machine à papier selon la revendication 7, **caractérisé en ce que** lesdites particules inorganiques comprennent des nanoargiles et/ou du SiC et/ou du carbure de bore.

10. Habillage de machine à papier selon l'une des revendications 7 à 9, **caractérisé en ce que** lesdites fibres inorganiques comprennent seules ou en association : du verre, du Kevlar ou du Nomex.

11. Habillage de machine à papier selon l'une des revendications précédentes, **caractérisé en ce** ladite structure matricielle comprend ledit matériau de charge (5, 14) dans la plage de 1 % en poids à 80 % en poids, de préférence de 1 % en poids à 50 % en poids, plus préférablement de 5 % en poids à 30 % en poids.

12. Habillage de machine à papier selon l'une des revendications précédentes, **caractérisé en ce** ladite structure matricielle comprend ledit matériau de charge fibreux (5) dans la plage de 5 à 20 % en poids, de préférence de 8 à 12 % en poids.

13. Habillage de machine à papier selon l'une des revendications précédentes, **caractérisé en ce** ladite structure matricielle comprend ledit matériau de charge particulaire (14) dans la plage de 5 à 50 % en poids, de préférence de 10 à 30 % en poids.

14. Habillage de machine à papier selon l'une des revendications précédentes, **caractérisé en ce que** ledit matériau de charge (5, 14) est mélangé de façon homogène dans ledit matériau matricielle polymère (4, 13).

15. Habillage de machine à papier selon l'une des revendications 1 à 14, **caractérisé en ce que** ladite structure matricielle comprend au moins une zone avec une teneur en matériau de charge (5, 14) supérieure comparativement aux autres zones.

16. Habillage de machine à papier selon l'une des revendications précédentes, **caractérisé en ce** ladite structure matricielle comprenant le matériau de charge (5, 14) possède un coefficient de dilatation thermique linéaire dans la plage de 1 x 10⁻⁵ K⁻¹ à 5 x 10⁻⁵ K⁻¹.

17. Habillage de machine à papier selon l'une des revendications précédentes, **caractérisé en ce que** ledit matériau de matrice polymère (4, 13) possède une température de fusion inférieure à la température de fusion desdits fils linéaires et/ou à la température de fusion dudit matériau de charge (5, 14).

18. Habillage de machine à papier selon l'une des revendications précédentes, **caractérisé en ce que** ledit matériau de matrice polymère (4, 13) comprend seul ou en association : un matériau thermoplastique ou élastomère thermoplastique tel qu'un polyester à base d'élastomère thermoplastique, un polyuréthane, un polyamide, un caoutchouc (organique ou inorganique).

19. Habillage de machine à papier selon l'une des revendications précédentes, **caractérisé en ce que** lesdits fils linéaires (2, 11) sont des fils monofilaments ou multifilaments, pliés ou torsadés ou filés-liés.

20. Habillage de machine à papier selon l'une des revendications précédentes, **caractérisé en ce que** lesdits fils linéaires (2, 11) comprennent un matériau inorganique.

21. Habillage de machine à papier selon l'une des revendications précédentes, **caractérisé en ce** ladite structure matricielle (3, 12) forme une surface plane sur au moins un côté de ladite toile non tissée.

22. Habillage de machine à papier selon l'une des revendications précédentes, **caractérisé en ce** ladite structure matricielle (3, 12) forme une surface texturée sur au moins un côté dudit habillage de machine à papier.

23. Habillage de machine à papier selon l'une des revendications précédentes, **caractérisé en ce que** ladite toile non tissée comprend des ouvertures (6) qui s'étendent au travers de ladite structure matricielle (3, 12).

24. Habillage de machine à papier selon la revendication 25, **caractérisé en ce que** lesdites ouvertures (6) sont uniformément espacées.

25. Habillage de machine à papier selon l'une des revendications 25 et 26, **caractérisé en ce que** lesdites ouvertures (6) sont dans une disposition décalée latéralement par rapport audits fils linéaires.

26. Habillage de machine à papier selon l'une des revendications 25 à 27, **caractérisé en ce que** lesdites ouvertures (6) sont des trous à parois droites ou des trous de forme conique.

27. Habillage de machine à papier selon l'une des revendications précédentes, **caractérisé en ce** ladite toile possède une perméabilité dans la plage de 20 pi³/min à 1000 pi³/min (9,43894 x 10⁻³ m³/s à 0,471947 m³/s).

28. Habillage de machine à papier selon l'une des revendications précédentes, **caractérisé en ce que** lesdites ouvertures (6) dans la structure matricielle (3, 12) comprennent des passages d'écoulement individuels essentiellement perpendiculaires au plan général de ladite toile.

29. Habillage de machine à papier selon l'une des revendications précédentes, **caractérisé en ce que** lesdits fils linéaires (2, 11) sont complètement intégrés dans ladite structure matricielle (3, 12).

30. Habillage de machine à papier selon l'une des revendications précédentes, **caractérisé en ce que** ledit habillage de machine à papier comprend une pluralité desdites toiles non tissées (1, 10) jointes ensemble d'une manière stratifiée et/ou côte à côte.

31. Habillage de machine à papier selon l'une des revendications précédentes, **caractérisé en ce qu'**au moins une surface de ladite toile non tissée est couverte d'une couche poreuse.

32. Habillage de machine à papier selon l'une des revendications précédentes, **caractérisé en ce que** ladite couche poreuse comprend une nappe textile.

33. Habillage de machine à papier selon l'une des revendications précédentes, **caractérisé en ce** ledit habillage de machine à papier est une toile de formation ou de séchage, un feutre coucheur ou une bande de couchage, une bande de lisse ou de transfert.

34. Procédé de fabrication d'un habillage de machine à papier avec une toile non tissée, le procédé comprenant les étapes de formation d'une structure matricielle qui comprend un matériau de charge et un matériau de matrice polymère et l'application de fils linéaires espacés se prolongeant essentiellement de manière parallèle les uns aux autres pendant ou après la formation de ladite structure matricielle à une étape de fusion dudit matériau de matrice polymère de telle manière par rapport à ladite structure matricielle que lesdits fils sont au moins en partie intégrés dans ladite structure matricielle et interconnectés par ladite structure matricielle.
